

Aug. 23, 1932.

J. J. QUINN

1,873,030

POWDER PUFF

Filed Dec. 26, 1930

2 Sheets-Sheet 1

*Fig. 1.*



*Fig. 2.*



*Fig. 3.*



Inventor:

John J. Quinn

By his Attorney

*A. R. Jones.*

Aug. 23, 1932.

J. J. QUINN

1,873,030

POWDER PUFF

Filed Dec. 26, 1930

2 Sheets-Sheet 2

*Fig. 4.*



Inventor:

John J. Quinn

By his Attorney

*A. R. Jones*

## UNITED STATES PATENT OFFICE

JOHN J. QUINN, OF SCARSDALE, NEW YORK, ASSIGNOR TO PINAUD, INC., OF NEW YORK,  
N. Y., A CORPORATION OF NEW YORK

## POWDER PUFF

Application filed December 26, 1930. Serial No. 504,729.

This invention relates to powder puffs and has for its object to provide a sanitary, inexpensive puff capable of carrying a substantial charge of powder and adapted to release such powder readily during a wiping operation. Another object is to provide a powder puff which is closer to the ideal needs than is any puff heretofore discovered.

There are many requirements for a powder puff, and among these may be mentioned the necessity for a soft powder carrying face with soft edges which are free of stitches, adhesive, or other material which is apt to scratch the face. The ideal puff should be so inexpensive as to allow its being used and then discarded. Heretofore various types of papers have been suggested but such materials are open to the objection of either not carrying enough powder or being too stiff. Another requirement is that while cheap it should nevertheless be capable of much longer use should the occasion demand as where the supply has been nearly exhausted away from a source of supply. Generally a puff is desired to have enough body or stiffness so that it will lie flat when not in use. As the vanity cases today are made quite thin and compact a powder puff that is adapted for use and carriage within such a case must also be quite thin. In addition to the ability of a puff to carry the desired charge of powder must be mentioned the ability to release or give up such charge of powder preferably on merely a wiping operation and without the necessity of patting since the latter is liable to spread excess powder over the clothes. Another reason for this last requirement is encountered with puffs which are inexpensive enough to be used and then discarded, because when discarding a puff it is preferred that no more powder be thrown away with the puff than is necessary. For this reason a puff which does not become readily impregnated with powder and which carries the desired charge on the surface where it may be released merely by wiping operations, will if it meets the other requirements mentioned constitute a much desired powder puff. The present invention satisfies all the foregoing

requirements more closely than has heretofore been possible.

Specifically this invention contemplates a powder puff of compressed absorbent cotton preferably having its back stiffened by a coating of starch or other material which if it works loose will not prove harmful to the face. While there have been prior art suggestions for the use of absorbent cotton powder puffs in several ways, these have all fallen short of meeting the foregoing requirements.

Referring to the drawings Fig. 1 shows a rear view of one embodiment of this invention.

Fig. 2 is a section on the line 2—2 of Fig. 1.

Fig. 3 is a face view of the puff shown in Figs. 1 and 2.

Fig. 4 is a graphical comparison between the puff of this invention and other commonly used powder puffs of the same size.

The powder puff 10 in Fig. 1 is of the general shape indicated and is provided on its back 12 with a plurality of longitudinally and laterally extending lines or impressions 13. Inwardly of its edge 15 is a border 14 in which the material has been compressed to a greater extent. The face 11 is of soft material well adapted to the foregoing requirements of a powder puff. In practice the absorbent cotton constituting this puff is compressed to about the thickness of an ordinary blotter, more frequently slightly thicker than sometimes thinner.

To form this puff a number of layers, in the present instance, seven layers, of well carded cotton are taken and compressed in sheets between rollers to about the thickness desired in view of the compression later. The sheets are then coated on one side with a liquid stiffening material such as starch and the like. The coated material is then passed between finishing rolls one of which has a surface adapted to give the longitudinal and lateral impression 13 in the stiffened back. These impressions serve to better bind the fibers together and while such impressions have in Fig. 1 been shown as forming the series of squares, it will nevertheless be understood that the same function may be at-

tained by the repetition of a series of letters or words indicating the maker or seller of the powder puff. While in sheet form and preferably before the starch material has dried the puffs may be cut out of the sheet to desired size by stamping. Preferably the stamping die is provided with a projection inwardly of the cutting edge so shaped as to substantially compress the border portion 14 to a much greater extent than the body portion of the puff has been compressed. This compressed border 14 serves the useful purpose of prolonging the life of the puff by reducing the tendency for the fibers to slide off or move over the edge of the puff either laterally or longitudinally during use. If desired the compressed border portions 14 can be formed while the material is in sheet form and prior to the stamping out operation.

In order to make the comparison between the compressed cotton puff of this invention and other commonly used puffs there were provided puffs of eiderdown, sheepskin, cotton velvet, wool velvet and compressed cotton of this invention, all of the same size namely,  $2 \times 2\frac{1}{2}$  centimeters in size. For each puff 25 milligrams of the same kind of powder was weighed out and placed in a depression surface similar to the wiping surface of those vanity cases whose wiping or discharge surface is separated or closed from the main body portion of the powder within the vanity case. The measured amount of powder was then taken up by each puff in a manner similar to the way in which powder is taken up on the puff in use. Each puff containing the powder was then gently wiped on a smooth skin (in each case the same skin) until no further powder was discharged from the puff, the skin being wiped with a towel after each stroke of a puff so as to be able to tell when no more powder was discharged. This is the end of what in Fig. 4 is called the first application and Fig. 4 shows that the powder puff of this invention discharged the greatest amount of powder and had the least amount of powder remaining on the puff, there being 13 milligrams of powder discharged and 12 remaining absorbed by the puff with the puff of this invention while the next best puff namely the wool velvet had 16 milligrams of powder left on the puff after this first application. The next best was the cotton velvet which had 17 milligrams of powder left on the puff while the eiderdown and sheepskin were equally poor in discharging only 4 milligrams, there being 21 milligrams left on each puff. From this much of the comparison it will be seen that the puff of this invention is much superior to any of the prior art puffs insofar as they are adapted to be used only once and then thrown away because after the first application of powder the puff of this invention discharged 52% of the quantity of powder it took up while

the next best discharged 36% and the cotton velvet puff discharged 32% and the sheepskin and eiderdown puffs each discharged only 8% of the powder taken up, leaving 92% of the powder taken up still left in the eiderdown and sheepskin puffs. Not only is the puff in this invention best suited and most efficient for delivering the greatest percentage of powder after a similar application of powder to the puff but the puff of this invention costs roughly about 1/30 the cost of the other puffs, which are all relatively expensive by comparison.

Fig. 4 also shows that with a second application of powder a puff of this invention still retained its lead over the others. For this second application another 25 milligrams of powder was weighed out and taken up by each puff in the same manner as before and the powder discharged from each puff by a wiping operation in the same manner as before. The powder applications were successively continued with the discharges until the curve for each material in Fig. 4 became substantially flat which indicates that the puff became substantially saturated because adapted to take up and give out the same amount of powder by a wiping operation. While the wool velvet puff became slightly more efficient after the third application of powder than the puff of this invention, the difference between the two from the standpoint of efficiency would be insignificant were it not for the tremendous difference in price of the wool velvet puff and the puff of this invention.

Among the advantages of this invention may be mentioned the superlative excellence of this puff to be used only once or more and then be thrown away. It is not the cost alone but also the ability of this puff to deliver a greater percentage of the powder taken up after one or two applications than is any other puff known. The reluctance to absorb or retain powder not only means economy in powder where puffs are to be used and then discarded, but this feature is also of importance in those newer vanity cases which have the powder discharge or wiping surface kept clean and free of powder and separated from the body of powder in the vanity case because where the puff contains less powder after being used there will be less likelihood of any powder retained by the puff being discharged upon the wiping surface of the vanity case whereby such surface may be given better insurance that it will be free of powder when the puff of this invention is used. Another feature of this invention comprises the stiffened integral back whereby no adhesive or other hard edges are formed and even if starch works loose from the back into the powder such will be harmless to the face because starch is one of the constituents of some face powders. Another advantageous fea-

ture of the present invention is the border 14 which is compressed to a greater extent than the rest of the puff. If it were not for this border there would be greater danger of some 5 of the fibers bodily shifting or moving off and over the edge of the puff with use. Therefore this border contributes to lengthen the life of this puff where such is necessary.

Other advantageous features include the 10 low cost to the puff of this invention and its soft face, soft edges, the safe and inexpensive back stiffening, and the adaptability of the present puff for carriage in the modern thin and compact vanity cases. This puff 15 may be sterilized and separately packed in envelopes of glassine paper and the like and sold in quantities at a price to make possible their being used only once or oftener if desired and then discarded. Such extreme 20 sanitary precautions would not be warranted with the older types of vanity cases where either the soiled puff of powder released from the soiled puff was brought in contact with and therefore free to contaminate the 25 main body portion of powder carried by the vanity case. A full scientific explanation of the reasons for the better efficiency of the puff of this invention over those of the prior art referred to is not clearly understood. A contributing cause may be that the fibers in this 30 new puff are generally parallel to each other and to the face of the puff, throughout the main body portion if not on the face. The other puffs analyzed have their fibers mostly 35 normal to the face of the puff although some have their fibers at various inclinations to the face of the puff, the eiderdown for example being principally fine feathers arranged at a variety of angles. On taking up powder 40 the puff of this invention appears to carry it more on the outside than on the inside of its face.

I claim:

1. A powder puff having a soft fibrous face 45 adapted to carry powder, edges which are substantially equally soft and a stiffened back of the same material as the face.
2. A compressed fibrous powder puff having a soft face and a back of stiffened face material.
3. A compressed absorbent cotton powder puff having a soft face and a back of stiffened face material.
4. A compressed fibrous powder puff having a soft face with the fibers in the body of the puff arranged substantially parallel with respect to each other and to the face of the puff and adapted when unimpregnated with powder to carry a substantial quantity of powder largely on the surface of said soft face and readily release during a wiping operation about half of the powder wiped up as a first charge.
5. A powder puff having soft fibrous face 85 adapted to carry powder largely on the out-

side of said face, edges which are substantially as soft as the face, and a stiffened back of the same material as the face and edges.

6. A compressed fibrous powder puff having a soft face with the fibers in the body of the puff arranged substantially parallel with respect to each other and to the face of the puff and adapted when unimpregnated with powder to carry a substantial quantity of powder largely on the surface of said soft face and readily release during a wiping operation a substantially larger percentage of the powder wiped up and carried as a first charge in use than any other puff.

7. A compressed fibrous powder puff having a soft face with the fibers in the body of the puff arranged substantially parallel with respect to each other and to the face of the puff and adapted when unimpregnated with powder to carry a substantial quantity of powder largely on the surface of said soft face and readily release during a wiping operation a substantially larger percentage of the powder wiped up and carried as a first charge in use than any puff having its face fibers extending substantially normally or angularly to the plane of such face, such as a puff of wool velvet, cotton velvet, sheepskin, eiderdown, or the like.

8. A powder puff thin enough for embodiment in a vanity case and being entirely of compressed absorbent cotton having one side stiffer than the other.

9. A compressed fibrous powder puff having a soft face with the fibers in the body of the puff arranged substantially parallel with respect to each other and to the face of the puff and being compressed to a substantially greater degree adjacent an edge portion than in the body of the puff, to reduce the tendency of the fibers to slide over the edge in wiping.

10. A powder puff of compressed absorbent cotton having the fibers adjacent an edge portion compressed to a substantially greater degree than are the fibers of the body portion of the puff.

11. A powder puff of compressed absorbent cotton having the fibers adjacent an edge portion compressed to a substantially greater degree than are the fibers of the body portion of the puff, the fibers which have been compressed to the greatest extent being inwardly of the edges which are compressed to no greater degree than are the fibers in the main body portion of the puff.

12. A powder puff of compressed absorbent cotton having its back coated with a stiffening material and imprinted with lines extending longitudinally and laterally of the fibers throughout the stiffened back to bind the fibers.

13. A powder puff of compressed absorbent cotton having its back coated with a stiffening material and imprinted with lines extending longitudinally and laterally of the

fibers throughout the stiffened back to bind the fibers, and a border which has been compressed to a greater extent than the body of the puff.

5. 14. A compressed fibrous powder puff having a soft face and a back of stiffened face material, the back of said puff being stiffened by contact with a liquid material which if it works loose when dry will not irritate the 10 skin, and which material has been used as a constituent of some face powders.

In witness whereof I have hereunto set my hand this 23rd day of December, 1930.

JOHN J. QUINN.

13

20

23

20

25

20

23

59

25

60

65